

Nov. 27, 1934.

E. G. FAHLMAN

1,982,423

MOLD AND METHOD OF CASTING

Filed May 2, 1932



Fig. 1.



Fig. 2.

INVENTOR  
*Everett G. Fahlman*  
BY *Evans & McCay*  
ATTORNEYS

## UNITED STATES PATENT OFFICE

1,982,423

## MOLD AND METHOD OF CASTING

Everett G. Fahlman, Cleveland, Ohio, assignor to  
 The Permold Company, Cleveland, Ohio, a  
 corporation of Ohio

Application May 2, 1932, Serial No. 608,715

4 Claims. (Cl. 22—212)

This invention relates to the casting of aluminum and alloys thereof, and more particularly to the casting of such metals in semi-permanent molds.

Many castings of aluminum or alloys thereof are formed in permanent molds, due to the advantages of this method of casting. In the case of certain castings having hollow interiors of more or less complex nature, however, frangible cores, such as of sand, are employed, the combination of sand core and metal mold parts being known as semi-permanent mold casting.

In the case of hollow castings of relatively thin section, where it has been desired to form solid lugs or similar heavy portions on the outer side of the casting directly adjacent to the thin section, great difficulties have been encountered due to the formation of sinks and cracks adjacent to the junction of the lug and thin casting section.

An object of this invention is to overcome the aforementioned difficulties and to provide a method of forming castings of aluminum or alloys thereof of widely varying sections in semi-permanent molds.

Another object is to provide a method of casting solid lugs on thin sections of hollow aluminum castings.

A further object is to provide an improved method of casting aluminum or alloys thereof in semi-permanent molds to form castings of intricate interior and of widely varying section.

Another object is to provide, for the semi-permanent mold type of casting aluminum and alloys thereof, an advantageous method of chilling uniformly the casting metal forming heavy and thin sections of the article being cast.

Other objects will be apparent to those skilled in the art from the disclosures herein made from the accompanying drawing, wherein

Figure 1 is a vertical section through a permanent mold and casting therein constructed according to the method outlined herein and through the frangible core cooperatively associated therewith; and

Fig. 2 is a horizontal section taken along the line 2—2 of Fig. 1.

The mold as shown somewhat diagrammatically is designed to cast a hollow object such as might be used as the cleaning nozzle of a vacuum cleaner and consists of a base plate 1 supporting the mold sections 2 and 3. These mold sections are recessed to form mating halves of a mold cavity 5 and 6 and also cooperatively recessed to form the pouring sprue cavity 7 and

gate 10. Mounted on the base plate 1 is the frangible core 8 which, with the mold cavity recesses 5 and 6 above mentioned, define a thin-walled, semi-cylindrical cavity with ends, such as might be used to cast the cleaning nozzle of a vacuum cleaner. It is, however, desired to cast on this thin-walled, hollow structure a heavy lug and the mold section 3 is accordingly provided with the recess 4 to form this lug.

There is provided, opposite the cavity for the lug 4, a recess in the sand core 9. This recess is thin and flat, being preferably about  $\frac{1}{16}$  inch in thickness for the casting shown in the drawing. Its area depends on the volume of metal to be cast into the lug 4. The recess is therefore usually comparatively narrow when it is desired to provide a casting having a lug such as described. In case of other heavy structures it may assume other forms, as will be later noted.

With the ordinary construction of a sand core it is found that a seriously large number of castings show imperfection in the form of cracks, sinks, etc. adjacent the base of the heavy lug. When, however, the sand core is provided with a recess as described, it is found that difficulties of this sort are largely or wholly overcome, and that in this way it is possible to cast heavy lugs on castings of generally thin section, and to produce generally perfect castings without the defects above mentioned. I do not here advance with certainty any explanation of this phenomenon. However, I believe it to be possibly due to the fact that the metal in the recess in the sand core cools more rapidly than does the metal in the thin section adjacent and much more rapidly than the metal in the heavy lug, and accordingly solidifies before the metal in either of the other two locations. The metal in the recess in the sand core being very thin, the relation of its area to volume is large and consequently it solidifies rapidly in spite of the low heat conductivity of the frangible core. When solidified, the conduction of heat through the thin chill is large and the chill conducts heat into a relatively large area of the frangible core and will therefore act as a solid metal chill to the rest of the casting at that point. In this way the metal of the lug is cooled as rapidly as is the metal of the thin section immediately adjacent, and the aforesaid sinks and cracks in and around this structure are prevented.

After the casting has solidified and the frangible core removed it is a very easy matter, owing to the thin cross section of the chill, to remove it if desired.

It will thus be seen that I have devised a method

- of chilling heavy sections of castings adjacent thin sections, which method is very much more easy to use than methods heretofore used for this purpose, and in which the chill is in a sense made integral with the casting and thereby has superior heat-conducting qualities therefrom. It will also be seen that it can be removed from the casting easily and that no defect in the surface or internal structure results thereby.
- 10 Due to its thin cross section and large area, the chill disclosed herein utilizes only a small amount of casting metal and its configuration is such that for purposes of description it may be termed a leaf chill.
- 15 While I have described and illustrated this invention as a method of forming heavy lugs on hollow castings of generally thin cross section, it is to be noted that the method is much more generally applicable. For example, the castings 20 may be flat though of thin cross section. Furthermore, the lugs or other thick cross section, the casting of which is to be facilitated, instead of being long and having a relatively small base attached to the casting as shown herein, may be 25 heavier and more than one leaf chill may be used. Instead of being in the form of a lug it may be of rib form, in which case either a number of leaf chills may be placed opposite it, or one or more long leaf chills may be provided running along 30 its axis on the other side of the thin section of the casting of adequate chilling effect for the rib or other heavy section to be cast.
- While the drawing describes a casting of a 35 generally hollow nature with a frangible core, this method is not limited thereto but is applicable to any semi-permanent mold where there are one or more thick sections adjacent to the thin sections.
- It will thus be seen that I have overcome in a 40 very simple manner a difficulty in the use of semi-permanent molds, which difficulty resides in the general problem of casting heavy sections adjacent thin sections, particularly when such thin section is defined by a frangible core of low heat 45 conductivity and of low specific heat. I have, by a very simple method, succeeded in increasing the apparent conductivity of such frangible mold members and utilizing a greater volume thereof for cooling purposes than ordinarily comes into 50 function. I have, moreover, provided what is in effect a chill which, through its integral character with the rest of the casting, has a great capacity for conducting heat away therefrom and which, through its thin cross section and large area, can 55 be easily removed, if desired, from the finished casting without marring the surface thereof, without using a great deal of metal, and without disturbing the internal structure of the casting.
- Furthermore, it is to be understood that the 60 particular forms of apparatus shown and described, and the particular procedure set forth, are presented for purposes of explanation and illustration and that various modifications of said

apparatus and procedure can be made without departing from my invention as defined in the appended claims.

What I claim is:

1. A semi-permanent mold comprising metal 80 mold members recessed to define the exterior wall of a molding cavity and a frangible core member within said cavity and defining the interior wall of the molding cavity, said mold members being formed to provide a cavity which is generally thin in cross section and which has a portion of relatively thick cross section, said frangible core member having a recess of thin cross section and relatively large surface area opening to the portion of the cavity of thick cross section.
2. A semi-permanent mold for producing castings composed of a relatively thin section and a relatively thick section comprising a metal mold member and a frangible mold member arranged in spaced relationship to each other to form a mold cavity having a comparatively thin cross section, said metal member being recessed to form a portion of the mold cavity for casting the thick section, and the frangible member having a relatively thin recess therein opposite to the recess of 100 the metal member in which the thick section is formed, to provide a space in which a relatively thin layer of metal may be cast in opposed relation to the thick section.
3. The process of forming castings having a 105 relatively thick section and a relatively thin section, which comprises arranging a metal mold member having a recess therein and a frangible mold member in opposed relationship to each other to define a mold cavity, casting metal in 110 said cavity to form the relatively thick and thin sections and simultaneously causing a portion of the casting metal to flow in a recess in the frangible mold member opposite the thick section having such a cross section that the metal in the 115 recess of the frangible mold will solidify before the metal in the thick section, and conducting heat from the thick section during the cooling thereof by means of the solidified metal formed in the frangible mold.
4. In the process of forming castings having a 120 relatively thick section and a relatively thin section in a semi-permanent mold in which a metal mold member forms the outer surface of the casting cavity and has a recess therein to form the 125 thick portion, and a frangible mold member forms the inner surface of the casting cavity, the steps which comprise pouring metal in the casting cavity to form the relatively thin and thick sections and simultaneously causing a portion of the 130 molten metal to flow into a narrow recess in the frangible member having such a cross section that metal in the recess will solidify before the metal in the thick section, and conducting heat from the metal in the thick section during the 135 solidification thereof by means of the solidified metal formed in the frangible mold.

EVERETT G. FAHLMAN.